

Sept. 3, 1957

H. A. ROBINSON ET AL

2,805,198

CATHODIC PROTECTION SYSTEM AND ANODE THEREFOR

Filed Feb. 29, 1956



Fig. 2

Fig. 1



Fig. 3

INVENTORS.  
Harold A. Robinson  
John J. Newport  
Oliver Osborn  
BY *Griswold & Burdick*  
ATTORNEYS

## 1

2,805,198

## CATHODIC PROTECTION SYSTEM AND ANODE THEREFOR

Harold A. Robinson, Midland, Mich., and John J. Newport and Oliver Osborn, Lake Jackson, Tex., assignors to The Dow Chemical Company, Midland, Mich., a corporation of Delaware

Application February 29, 1956, Serial No. 568,619

8 Claims. (Cl. 204—197)

This invention relates to a cathodic protection anode formed of a galvanically active metal and to a cathodic protection system wherein such a protection anode is employed.

Cathodic protective anodes have been used for many purposes, such as preventing corrosion of structures in sea water, pipelines buried in the soil and internal areas of hot water heaters. For the most part, these anodes are made of readily expendable magnesium which has been alloyed with other metals to give the anode properties which particularly adapt it for its intended use. For example, cell magnesium has a satisfactory solution potential, but a poor current efficiency. Certain magnesium alloys have improved current efficiencies, but lower solution potentials than cell magnesium. Consequently, more alloy anodes are required to protect a given structure, but under predetermined conditions of use these anodes will have a longer useful life. Offsetting to a certain extent some of the advantages of these anodes made from magnesium alloy is the cost of the additional process steps and alloying ingredients.

It is an object of this invention to provide an improved cathodic protection anode composed essentially of magnesium and containing minor amounts of manganese and aluminum present in a predetermined ratio to each other. Another object of this invention is to provide an improved system for cathodically protecting structures immersed in media in which they are subject to corrosion. Still another object of this invention is to provide a process for making an improved cathodic protection anode directly from the melt in cell in which the magnesium metal is first prepared.

It has been discovered that an improved cathodic protection anode is obtained by forming the anode from a magnesium base alloy containing from 0.50 to 1.3 percent by weight manganese and not more than 0.010 percent by weight aluminum. A preferred method of making these anodes is to add a suitable manganese compound to the feed of a magnesium electrolytic cell, and the preferred composition comprises from 0.50 to .80 manganese and not over 0.005 aluminum (in weight percent), with the balance essentially magnesium. When such anodes are employed in a system for cathodically protecting structures composed of a metal less anodic than magnesium, they have a greatly improved current efficiency combined with an unusually high solution potential. These systems are thus advantageous in that they require fewer anodes and have a longer life than cell magnesium anodes, for example.

The present invention is useful in providing cathodic protection for structures immersed in sea water, and can be used under some conditions as a protective anode in hot water heaters. Yet anodes and systems comprising

## 2

ing the present inventions achieve their ultimate utility in protecting metal structures buried in high resistivity soils (above 1,500 ohms/cm.<sup>3</sup>). In hot water heaters, the galvanic cell created by the magnesium anode frequently encounters low resistance in the electrolyte present, so that a correspondingly high current is generated at a given voltage or potential. Consequently, an anode metal having relatively low solution potential is desirable to avoid useless current generation which is in turn accompanied by rapid consumption of the anode metal. When the structure to be protected is buried in high resistance soil, this high resistance so reduces the current flowing through the soil from the anode to the corrodible structure that a high voltage or anode solution potential is needed to adequately protect the structure. The all-around adaptability of the anode and the cathodic protective system comprising the present invention is manifested by the fact that it retains its high current efficiency and solution potential in sea water, saline soils and non-saline soils where the anode usually operates in a sulfate rich backfill.

Anodes comprising the present invention have the following composition in percent by weight:

|                     |                 |
|---------------------|-----------------|
| Magnesium           | At least 98.5.  |
| Manganese           | 0.50 to 1.3.    |
| Aluminum            | Not over 0.010. |
| Iron                | .001 to 0.03.   |
| Tin                 | Not over 0.01.  |
| Nickel              | Not over .002.  |
| Lead                | Not over 0.01.  |
| Other metals (each) | Not over 0.05.  |

In the electrolytic production of magnesium, the molten magnesium in the electrolytic cell is referred to as "cell magnesium." Essentially, cell magnesium is pure magnesium, but certain adventitious elements are present in small amounts. In the production of anodes comprising the present invention, amounts of these adventitious elements must be controlled. Iron is present in at least 0.001 percent by weight and must be limited to a maximum of 0.03 percent if an anode of the desirable characteristics of the present invention is to be obtained. Nickel is restricted to not over 0.002 percent by weight and the tin and lead should not exceed 0.01 percent. The other metals present do not exceed 0.05 percent each. The total of all such adventitious elements does not exceed 0.2 percent in the cell magnesium.

Aluminum is always present in small amounts in cell magnesium and will vary from 0.0001 up to 0.02 weight percent. Although it has previously been recognized that high percentages of iron were detrimental in anodes used for cathodic protection, little if any attention was directed to the amount of aluminum in the cell magnesium. It has now been found that the current efficiency of anodes made from cell magnesium is closely related to the amount of aluminum present. With larger amounts of aluminum, i. e. over .005 weight percent, the current efficiency of the anode drops drastically.

It has been discovered that by adding manganese to the cell magnesium in an amount definitely related to the amount of aluminum present, an alloy is produced which, when made into anodes, combines an even higher solution potential than cell magnesium with a high current efficiency. Measuring current efficiency in ampere hours per pound of anode metal, cell magnesium anodes usually fall between 200 and 300 hours per pound. Anodes comprising the present invention, on the other hand, will

have current efficiencies of at least 400 and as high as 565 hours per pound. Although the exact reason for this remarkable increase in current efficiency is not known, it is believed that the manganese in some way ties up or counteracts the detrimental effects of the iron-aluminum phase which is known to adversely affect the current efficiency of the anodes.

The solution potential of anodes comprising the present invention is substantially uniform when the manganese content is at least 0.5 percent and not over 1.3 percent by weight. Above and below these values, however, the solution potential does decrease. In this same range, the amount of manganese is adjusted relative to the amount of aluminum present to obtain enhanced current efficiency and the highest solution potentials. Figure 1 illustrates the critical effect of the Mn/Al ratio on the current efficiency of the anode by plotting test data from alloys comprising the present invention which have similar aluminum content on a graph in which the ordinates represent ampere hours per pound of anode metal and the abscissas represent the percent by weight of manganese. The details of the tests and data upon which Figure 1 is based are set forth in Examples 1 and 2 below.

It is apparent from Figure 1 that the low aluminum alloys (less than .001 percent) have consistently good current efficiencies when between 0.5 percent and 1.3 percent by weight of manganese is present. As the amount of aluminum increases, the decrease in current efficiency becomes more pronounced in the lower ranges of manganese content. Higher percentages of manganese result in satisfactory efficiencies for all aluminum contents not over .01%. It is thus seen that the ratio of manganese to aluminum is the critical factor. Since it is desirable to know how little manganese can be added and still overcome the detrimental effect of the aluminum, an empirical formula based on the data from the following Example 2 shows that the percent by weight of manganese added must be at least equal to  $0.5 + 60$  (percent by weight of aluminum present). Thus, for an aluminum content of .004 percent the minimum manganese content is  $0.5 + 60(0.004) = 0.5 + .24 = 0.74$  percent by weight. When the aluminum concentration equals 0.01 percent, the minimum amount of manganese required is  $0.5 + 60(0.01) = 0.5 + 0.6 = 1.1$  percent.

It should be pointed out that the experimental data of the examples were obtained under conditions simulating high resistivity soils at a current density of 36 milliamperes per square foot. In low resistivity or sea water environment, where the current may be many times greater, less manganese may be required to give enhanced current efficiency and maximum solution potentials. In no case, however, will the minimum amount of manganese required be less than 0.5 percent.

An alloyed anode of the type comprising the present invention can be produced by numerous means, such as treatment of cell magnesium in a separate alloying pot. The preferred manner of producing such alloyed anodes, however, comprises adding a manganese compound, such as manganese dioxide or manganese dichloride, to the feed of an electrolytic cell for making magnesium. The constituents of the cell are analyzed at frequent intervals and the manganese added in the feed is adjusted according to the aluminum content of the cell magnesium. In this connection it is important to note that manganese is an expensive alloying metal and minimum amounts useable are employed to reduce the cost of these sacrificial anodes, which may be employed to the extent of several tons for uses such as protecting pipelines. The casting of anodes from this alloy follows the conventional procedures, although it is preferred to employ relatively cool molds.

In order to enable those skilled in the art to more readily practice the present invention, the following examples are set forth to illustrate the present invention:

#### Example 1

The melt in a magnesium cell was analyzed by a direct reading spectrophotometer and found to contain by weight, .0052 percent Al, .0013 percent Cu, .014 percent Fe, less than .01 percent Ca, less than .0005 percent Ni, less than .001 percent Pb, less than .001 percent Si, less than .01 percent Sn, less than .02 percent Zn, and the balance magnesium. To the feed in this cell was added enough manganese dioxide to produce in the melt a minimum of 0.81 percent by weight of manganese ( $0.5 + 60(0.0052) = 0.5 + 0.31$ ). Final analysis showed 0.92 weight percent of manganese.

From this melt, magnesium anodes used for laboratory investigations were cast in iron molds just slightly over 100° C. and immediately air cooled to room temperature. These anodes were prepared by sectioning specimens roughly 7 inches long and  $\frac{1}{2}$  inch square cross section from 17 pound D-shaped production anodes. These specimens were machined to give small rods,  $\frac{5}{16}$  inch in diameter by 6 inches long. A 2 inch section at one end of each rod was threaded and a flat was filed near the middle of the threaded section to allow for the stamping of identification numbers. After weighing, the threaded section was smeared lightly with petroleum grease and the anode was then screwed into a transparent sleeve, threaded at the lower end to take the anode. The 4-inch length of anode extending beyond the grease-sealed sleeve was then vapor-degreased with trichlorethylene.

Employing the anodes so prepared, experimental cells were assembled using a 5.5 inch length of 3.5 inch standard pipe for the cathode, and an aqueous solution saturated with  $\text{CaSO}_4$  and  $\text{Mg}(\text{OH})_2$  interposed between the rod and the cathode in the electrolyte. This cell was then connected in series with other test cells and operated at an anode current density of 36 milliamperes per square foot for 14 days. The anodes were then removed from the cells and the loose corrosion product was brushed or rubbed off in a stream of running water. This was followed by immersion in agitated, aqueous 20 percent chromic acid solution, containing 1 percent  $\text{AgNO}_3$ , to remove residual corrosion products, after which the anodes were rinsed, dried and reweighed. Current efficiencies were calculated from the weight loss and the quantity of current passed. On this basis, this anode showed a current efficiency of 521 ampere hours per pound of anode metal.

#### Example 2

A series of tests following the procedures above outlined were made and the results of these tests formed the basis for Figure 1. The alloy in each case contained approximately .0005 percent Cu, less than .01 percent Ca, less than .0005 percent Ni, less than .001 percent Pb, less than .001 percent Si, less than .01 percent Sn and less than .02 percent Zn, with the balance magnesium except for aluminum, iron and manganese as tabulated.

In addition to the current efficiency test above outlined in Example 1, these same test anodes were tested for solution potential by immersion, following the current efficiency test, in an aqueous solution saturated with  $\text{CaSO}_4$  and  $\text{Mg}(\text{OH})_2$ , and allowed to soak for one hour. The samples were then connected to a calomel electrode with a saturated potassium chloride salt bridge and their solution potentials determined without removal of the specimens from the test solution. The following table shows a number of alloys tested both for current efficiency and solution potential, each of these alloys having a composition as set forth above, except for the variations in the amount of aluminum, iron and manganese as noted. To parallel Figure 1, the data is arranged according to the aluminum content, each set of data constituting an average of three test specimens. Alloys falling outside the prescribed range of manganese have been included to show the criticality of the manganese content.

| Percent by Weight of metals |            |            | Amp. Hours per pound of Anode Metal | Open Circuit solution potential ref: calomel |
|-----------------------------|------------|------------|-------------------------------------|----------------------------------------------|
| Percent Al                  | Percent Fe | Percent Mn |                                     |                                              |
| .0005                       | .008       | .70        | 557                                 | 1.665                                        |
| .0005                       | .013       | .84        | 520                                 | 1.647                                        |
| .0005                       | .012       | .86        | 516                                 | 1.644                                        |
| .0005                       | .0116      | .99        | 449                                 | 1.622                                        |
| .0006                       | .0107      | 1.20       | 523                                 | 1.664                                        |
| .0007                       | .0091      | .80        | 543                                 | 1.654                                        |
| .0008                       | .0163      | .77        | 536                                 | 1.646                                        |
| .0008                       | .0050      | .84        | 548                                 | 1.646                                        |
| .0008                       | .0055      | .85        | 529                                 | 1.624                                        |
| .0008                       | .0118      | .87        | 479                                 | 1.653                                        |
| .0008                       | .005       | .90        | 563                                 | 1.672                                        |
| .0008                       | .0059      | .92        | 532                                 | 1.649                                        |
| .0008                       | .0107      | .97        | 544                                 | 1.654                                        |
| .0009                       | .010       | .61        | 468                                 | 1.629                                        |
| .0009                       | .010       | .73        | 518                                 | 1.650                                        |
| .0009                       | .009       | .78        | 503                                 | 1.672                                        |
| .0009                       | .0145      | .80        | 527                                 | 1.638                                        |
| .0009                       | .0086      | .84        | 520                                 | 1.655                                        |
| .0009                       | .0062      | .86        | 540                                 | 1.633                                        |
| .0010                       | .0066      | .85        | 550                                 | 1.656                                        |
| .0011                       | .017       | .86        | 520                                 | 1.634                                        |
| .0011                       | .0086      | .86        | 486                                 | 1.638                                        |
| .0012                       | .0094      | .81        | 520                                 | 1.639                                        |
| .0013                       | .016       | .45        | 355                                 | 1.628                                        |
| .0013                       | .014       | .74        | 483                                 | 1.635                                        |
| .0013                       | .0074      | .76        | 498                                 | 1.642                                        |
| .0013                       | .007       | .77        | 542                                 | 1.675                                        |
| .0013                       | .0072      | .82        | 538                                 | 1.655                                        |
| .0014                       | .0084      | .97        | 498                                 | 1.647                                        |
| .0015                       | .015       | .68        | 460                                 | 1.666                                        |
| .0016                       | .020       | .64        | 400                                 | 1.637                                        |
| .0016                       | .012       | .69        | 461                                 | 1.628                                        |
| .0016                       | .013       | .72        | 495                                 | 1.661                                        |
| .0016                       | .009       | .85        | 489                                 | 1.635                                        |
| .0016                       | .0074      | .91        | 528                                 | 1.641                                        |
| .0017                       | .0076      | .74        | 498                                 | 1.633                                        |
| .0017                       | .0046      | 1.01       | 560                                 | 1.644                                        |
| .0019                       | .018       | .72        | 448                                 | 1.634                                        |
| .0019                       | .017       | .74        | 507                                 | 1.654                                        |
| .0019                       | .0067      | .82        | 486                                 | 1.628                                        |
| .0019                       | .0096      | 1.32       | 548                                 | 1.642                                        |
| .0020                       | .014       | .81        | 527                                 | 1.641                                        |
| .0022                       | .015       | .65        | 443                                 | 1.634                                        |
| .0022                       | .0107      | .72        | 450                                 | 1.644                                        |
| .0023                       | .012       | .68        | 438                                 | 1.627                                        |
| .0023                       | .0082      | .91        | 508                                 | 1.640                                        |
| .0024                       | .016       | 1.20       | 546                                 | 1.651                                        |
| .0025                       | .005       | .78        | 413                                 | 1.668                                        |
| .0025                       | .0068      | 1.29       | 541                                 | 1.626                                        |
| .0027                       | .019       | .77        | 451                                 | 1.643                                        |
| .0028                       | .0072      | .73        | 442                                 | 1.625                                        |
| .0028                       | .0113      | .76        | 402                                 | 1.638                                        |
| .0028                       | .009       | .89        | 567                                 | 1.661                                        |
| .0034                       | .0064      | .72        | 398                                 | 1.629                                        |
| .0034                       | .0040      | 1.06       | 507                                 | 1.624                                        |
| .0035                       | .0096      | .84        | 466                                 | 1.648                                        |
| .0035                       | .0140      | .90        | 507                                 | 1.629                                        |
| .0042                       | .0091      | .96        | 509                                 | 1.652                                        |
| .0045                       | .015       | .51        | 202                                 | 1.668                                        |
| .0045                       | .0159      | .76        | 438                                 | 1.644                                        |
| .0052                       | .014       | .92        | 521                                 | 1.665                                        |
| .0055                       | .010       | .65        | 298                                 | 1.627                                        |
| .0055                       | .0098      | .70        | 347                                 | 1.658                                        |
| .0067                       | .0110      | .63        | 223                                 | 1.631                                        |
| .0097                       | .0092      | 1.13       | 567                                 | 1.626                                        |
| <.03                        | .012       | 1.71       | 508                                 | 1.554                                        |
| <.03                        | .011       | 2.06       | 515                                 | 1.590                                        |
| <.03                        | .009       | 2.48       | 450                                 | 1.585                                        |
| <.03                        | .014       | 1.36       | 517                                 | 1.592                                        |
| .0012                       | .031       | .05        | 236                                 | 1.590                                        |
| .0008                       | .029       | .07        | 205                                 | 1.586                                        |
| .0008                       | .019       | .08        | 163                                 | 1.585                                        |
| .0002                       | .024       | .08        | 279                                 | 1.591                                        |
| .0002                       | .024       | .08        | 310                                 | 1.597                                        |
| <.03                        | .020       | .12        | 90                                  | 1.598                                        |
| .0003                       | .030       | .15        | 179                                 | 1.593                                        |
| .0047                       | .023       | .17        | 97                                  | 1.599                                        |
| .0002                       | .026       | .19        | 375                                 | 1.605                                        |
| .0004                       | .026       | .25        | 390                                 | 1.635                                        |

The data from this table relating to solution potential are plotted in Figure 2, which graphically shows high solution potentials between 0.5 and 1.3 percent manganese with rather sharp decreases in solution potential above and below these points. It is thus seen that the alloys of the above table which fall within the scope of the present invention combine a high current efficiency with a high solution potential.

In order to describe the cathodic protection system comprising the present invention, reference is made to Figure 3, which is a schematic illustration of an anode field positioned about a bare ferrous metal pipeline, in this case, a bare metal 8 inch diameter pipe which is to be protected. The pipeline 1 is connected through an insu-

lated electrical conductor 2 to an insulated collector wire 3, so-called because it interconnects through lead wires 4-4 with anodes, 5-5. These anodes, which are formed from the alloy above described, may be of various sizes,

5 but are in this instance 4 inches by 20 inches and are spaced at least 10 feet from the pipeline 1 and from 50 to 75 feet from each other. These anodes operate most efficiently and have a longer life when surrounded by a backfill 6-6. For high resistivity soils, the backfill 6 may 10 be composed of 20 parts bentonite (dry, powdered), 75 parts gypsum (dry, powdered) and 5 parts sodium sulfate (anhydrous). This backfill isolates the anode chemically and acts as an electrolytic bridge carrying electricity from anode to earth.

15 For most installations, anodes need be used only on one side of the pipeline to be protected, although exceptionally large pipes may require anodes on both sides. The spacing of the anodes in the station shown in Figure 3, as well as the total number of stations required, is a

20 function of the solution potential of the anode, the resistivity of the soil and the amount of current required to protect the pipeline. Other factors being equal, anodes of the present invention which have higher solution potentials than those of the prior art, may be spaced farther 25 apart, thus reducing the total number of anodes needed. Those skilled in the art will recognize that the distances, size of anodes, etc. shown in Figure 3 may be varied to suit the particular conditions encountered.

It is apparent from the above detailed description of 30 the invention that a cathodic protection anode has been produced which, when utilized in a cathodic protection system, is characterized by remarkable current efficiency combined with high solution potential. These results are obtained by restricting the alloy composition of the anode 35 within very narrow and critical ranges and particularly by maintaining the ratio of manganese to aluminum at a prescribed minimum. The invention is especially adapted for use in high resistivity soils, wherein a high solution potential is needed.

40 What is claimed is:

1. A cathodic protection anode formed of galvanically active metal having the following composition in percent by weight:

45 Magnesium ----- At least 98.5.  
Manganese ----- 0.50 to 1.3.  
Aluminum ----- Not over 0.01.  
Tin ----- Not over 0.01.  
Lead ----- Not over 0.01.  
50 Iron ----- 0.001 to 0.03.  
Nickel ----- Not over 0.002.  
Other metals (each) ----- Not over 0.05.

the amount of manganese in weight percent being at least 55 equal to 0.5+60 (percent by weight of aluminum).

2. A cathodic protection anode formed of a cast body of galvanically active metal having the following composition in percent by weight:

60 Magnesium ----- At least 99.16.  
Manganese ----- 0.5 to 0.8.  
Aluminum ----- Not over 0.005.  
Iron ----- 0.001 to 0.03.  
Nickel ----- Not over 0.002.  
65 Tin ----- Not over 0.01.  
Lead ----- Not over 0.01.  
Other metals (each) ----- Not over 0.05.

the amount of manganese in weight percent being at least 70 equal to 0.5+60 (percent by weight of aluminum).

3. In combination with a structure composed of corrodible metal less anodic than magnesium immersed in a medium wherein it is corrodible, a protective system of sacrificial metal submerged in the corrodible medium and 75 electrically connected to said structure and comprising

an expendable quantity of magnesium metal having the following composition in percent by weight:

|                     |                 |
|---------------------|-----------------|
| Magnesium           | At least 98.5.  |
| Manganese           | 0.50 to 1.3.    |
| Aluminum            | Not over 0.01.  |
| Tin                 | Not over 0.01.  |
| Lead                | Not over 0.01.  |
| Iron                | 0.001 to 0.03.  |
| Nickel              | Not over 0.002. |
| Other metals (each) | Not over 0.05.  |

the percent by weight of manganese being at least equal to  $0.5 + 60$  (percent by weight of aluminum).

4. The combination defined in claim 3 wherein the corroding medium is sea water.

5. The combination defined in claim 3 wherein the corroding medium is a soil.

6. In combination with a structure composed of ferrous metal immersed in a high-resistivity soil, a protective system of sacrificial metal submerged in the high resistivity soil and electrically connected to said structure so as to form a galvanic cell therewith, and comprising an expendable quantity of a magnesium alloy having the following composition in percent by weight:

|                     |                 |
|---------------------|-----------------|
| Magnesium           | At least 98.5.  |
| Manganese           | 0.50 to 1.3.    |
| Aluminum            | Not over 0.01.  |
| Tin                 | Not over 0.01.  |
| Lead                | Not over 0.01.  |
| Iron                | 0.001 to 0.03.  |
| Nickel              | Not over 0.002. |
| Other metals (each) | Not over 0.05.  |

the amount of manganese in weight percent being at least equal to  $0.5 + 60$  (percent by weight of aluminum).

7. A method of cathodically protecting a structure composed of a corrodible metal less anodic than magnesium immersed in a medium wherein it is corrodible, which comprises placing a protective system of sacrificial metal in the corroding medium composed of an expendable quantity of magnesium alloy having the following composition in percent weight:

|                     |                 |
|---------------------|-----------------|
| Magnesium           | At least 98.5.  |
| Manganese           | 0.50 to 1.3.    |
| Aluminum            | Not over 0.01.  |
| Tin                 | Not over 0.01.  |
| Lead                | Not over 0.01.  |
| Iron                | 0.001 to 0.03.  |
| Nickel              | Not over 0.002. |
| Other metals (each) | Not over 0.05.  |

10 the amount of manganese in weight percent being at least equal to  $0.5 + 60$  (percent by weight of aluminum), and electrically connecting said structure and the sacrificial metal to produce a galvanic cell in which the sacrificial metal is the anode and the structure is the cathode.

8. A cathodic protection anode formed of galvanically active metal having the following composition in percent by weight:

|                     |                 |
|---------------------|-----------------|
| Magnesium           | At least 98.5.  |
| Manganese           | 0.50 to 1.3.    |
| Aluminum            | Not over 0.01.  |
| Tin                 | Not over 0.01.  |
| Lead                | Not over 0.01.  |
| Iron                | 0.001 to 0.03.  |
| Nickel              | Not over 0.002. |
| Other metals (each) | Not over 0.05.  |

20 the amount of manganese in weight percent being at least equal to  $0.5 + 60$  (percent by weight of aluminum) when the percent by weight of aluminum exceeds .007.

#### References Cited in the file of this patent

#### UNITED STATES PATENTS

|           |              |               |
|-----------|--------------|---------------|
| 1,960,700 | Gann et al.  | May 29, 1934  |
| 2,431,723 | Yerkes       | Dec. 2, 1947  |
| 2,478,479 | Grebe et al. | Aug. 9, 1949  |
| 2,645,612 | Taylor       | July 14, 1953 |
| 2,698,230 | Boyle        | Dec. 28, 1954 |
| 2,742,355 | Emley        | Apr. 17, 1956 |

#### OTHER REFERENCES

40 H. H. Robinson, Transactions of the Electrochemical Society, vol. 90 (1946), pp. 496-499.